

# United States Patent

Brault et al.

[15] 3,642,478

[45] Feb. 15, 1972

[54] **PROCESSES AND COMPOSITIONS FOR CONVERTING ZERO VALENT METALS PHOTOGRAPHIC IMAGES TO FORMAZAN DYE IMAGES**

- [72] Inventors: **Albert T. Brault, Rochester, Vernon L. Bissonette, Brockport, both of N.Y.**
- [73] Assignee: **Eastman Kodak Company, Rochester, N.Y.**
- [22] Filed: **Feb. 25, 1970**
- [21] Appl. No.: **14,228**

- [52] U.S. Cl. .... **96/48, 96/51, 96/60 BF**
- [51] Int. Cl. .... **G03c 5/24, G03c 5/44**
- [58] Field of Search..... **96/60 R, 60 BF, 48, 51**

[56] **References Cited**

UNITED STATES PATENTS

- 3,503,741 3/1970 Wilson et al. .... **96/20**
- 3,414,411 12/1968 Michel et al. .... **96/29 D**

FOREIGN PATENTS OR APPLICATIONS

670,883 4/1952 Great Britain ..... **96/54**

*Primary Examiner*—Norman G. Torchin  
*Assistant Examiner*—Alfonso T. Suro Pico  
*Attorney*—W. H. J. Kline, J. R. Frederick and R. C. Livermore

[57]

**ABSTRACT**

A zero valent metal image in which the metal has a standard oxidation potential more positive than -0.98 volt is advantageously replaced by a formazan dye by the single process step of contacting the metal image with a solution of a ligand in the presence of a tetrazolium salt when the combination of tetrazolium salt and ligand with water and zero valent metal produces a solution reaction potential E greater than  $\pm 0.01$  volt, the process forming a good dye image when the formazan dye is nondiffusible and the process blixing the metal image when the formazan dye is diffusible and the metal-ligand complex is diffusible. Compositions of tetrazolium salt and ligand are advantageously used in this single step process for dye image formation or for blixing a metal image.

20 Claims, No Drawings

PROCESSES AND COMPOSITIONS FOR CONVERTING  
ZERO VALENT METALS PHOTOGRAPHIC IMAGES TO  
FORMAZAN DYE IMAGES

This invention is related to photography, compositions for use in photographic processing, photographic processes for forming dye images and processes for the removal of metal images and metal salts from a color-developed color photographic element.

In the photographic processing of certain color photographic elements, silver images and dye images are formed during the color development step or steps, and it is desired to remove the silver image and any residual silver halide so that the processed element will contain only the dye images and will not be subject to the formation of printout of silver from residual silver halide upon prolonged exposure to viewing light. The silver image is usually bleached, i.e., converted to a silver salt by treating it, for example, with a solution of alkaline metal ferricyanide in the presence of bromide ions, and then subsequently treating the silver salt with a silver salt complexing agent, such as an alkaline metal thiosulfate solution to convert the silver salt into a water-soluble, diffusible complex which is readily removed by washing the photographic element.

Alternatively, the silver and residual silver halide can be removed by using a blix, i.e., combined bleach-fix solution. Farmer's Reducer, formed by combining a solution of water-soluble ferricyanide and a water-soluble thiosulfate, is a strong blix; however, it has a very short life and, for this reason, is not practical for many color processing applications. Other well-known blixes use, as an oxidizing or bleaching agent, a ferric ion EDTA complex with a thiosulfate fixing agent. Although this type of blix is quite effective in removing the silver and silver halide from the color-processed element, it is quite frequently necessary to use a separate bleach bath in addition to the blix in order to insure that leuco forms of certain dye images formed during color processing are completely converted to the colored or dye form. It is therefore desirable to provide other blix compositions which are stable and which can be used without the necessity of having a separate bleach bath.

British Pat. No. 908,299 describes a process for converting a silver image in a photographic emulsion layer into a formazan dye image by treating the silver image with a tetrazolium salt in the presence of cyanide ions, and subsequently bleaching with a ferricyanide bromide bleach bath, followed by washing, fixing with a sodium thiosulfate bath, washing and drying. The use of cyanide ion is very undesirable because of the danger to the operating personnel. Furthermore, the process described by the British patent requires a separate, additional bleach, fix and three intermediate washing steps in order to remove the silver image left after forming the formazan dye image.

It is therefore an object of our invention to provide a novel blix composition which is stable and is valuable for use in color photographic processing.

Another object of our invention is to provide a novel process for removing silver and residual silver halide from a color-developed photographic element.

Another object of our invention is to provide a novel process for converting a metal image to a formazan dye image and, simultaneously, to remove the metal image from a black-and-white developed photographic element.

Still another object of our invention is to provide a novel composition which is valuable for the conversion of a silver image into a formazan dye image and, simultaneously, to remove the silver image in a single process step.

Still other objects of our invention will become apparent from a consideration of the following specification and claims.

These and still other objects of our invention are accomplished by the preparation and use of our novel combina-

tions comprising (1) a tetrazolium salt (T-salt), (2) a ligand which forms a soluble and diffusible metal complex, (3) water and (4) a zero valent metal that has a standard oxidation potential more positive than -0.98 volt such that our combination produces a solution reaction potential E of at least +0.01 volt. The components in our novel combination react to produce a formazan dye and a metal compound that is in equilibrium with a very low concentration of the metal ions. In one embodiment of our invention, substantially all of a metal image is converted to (i.e., replaced by) a nondiffusible formazan dye image by contacting said metal image with an aqueous solution of a ligand that forms a soluble and diffusible metal complex in the presence of a T-salt and substantially all of the metal image is complexed without the need for a separate bleach step followed by a washing step and a separate fix step as is required by the prior art. Our process can advantageously be used to replace at least a part or all of a metal image with a formazan dye image. Water-soluble and diffusible T-salts (i.e., a T-salt whose solution will pass freely to said metal image when it is in a colloid layer) are advantageously included in the same aqueous solution with said ligand.

In another embodiment of our invention, compositions comprising (1) a water-soluble and diffusible T-salt that is reduced by metal to form a water-soluble and diffusible formazan dye and (2) a water-soluble and diffusible metal complexing agent that forms a water-soluble and diffusible metal complex, are dissolved in water to make blix solutions that are valuable for removing silver and silver halide from color-developed color photographic elements.

The solution reaction potential E is defined as follows:

$$E = (E^{\circ} M^{\circ} \rightarrow M^{m+}) - (E^{\circ} \text{Form} \rightarrow \text{T-salt}) - \frac{0.059}{d} \log \frac{[M^{m+}]^a [Formazan]^b}{[T\text{-salt}]^b [H^+]^b}$$

in which a and b are each integers of from 1 to 3 determined by the stable oxidation state of metal ion and which are needed to satisfy the stoichiometric relationship of the reaction of metal with T-salt; d represents the number of electrons transferred in said reaction;

$$E^{\circ} M^{\circ} \rightarrow M^{m+} \text{ and } E^{\circ} \text{Form} \rightarrow \text{T-salt}$$

are the standard oxidation potentials for (1) zero valent metal to metal ion of valence m and (2) formazan dye to T-salt, respectively,  $[M^{m+}]$ ,  $[\text{Formazan}]$ ,  $[\text{T-salt}]$  and  $[H^+]$  represent the concentrations of the indicated material. Standard oxidation potentials are for unit activity at 25° C. as referred to the hydrogen-hydrogen ion couple as zero volts. (See Handbook of Chemistry & Physics, 41st Edition, page 1,733 (1959).)

The water-soluble, diffusible tetrazolium salts used to advantage according to our invention, are represented by the following formulas;



wherein  $R_1$  and  $R_3$  each represent a group such as an aryl group, a phenyl group (e.g., phenyl, tolyl, butylphenyl, a hydroxyphenyl group, an alkali metal or ammonium salt of

Carboxyethylphenyl, a carboxyethylphenyl group, an ethoxy carbonylphenyl group, an aminophenyl group, a carbamylphenyl group, a sulfoethylphenyl group, an alkali metal or ammonium salt of a sulfonylphenyl group, a sulfonamidophenyl group, a sulfamylphenyl group, a mercaptophenyl group, a nitrophenyl group, etc.), a naphthyl group (e.g.,  $\alpha$ -naphthyl,  $B$ -naphthyl, a carboxynaphthyl group, a hydroxynaphthyl group, a sulfonaphthyl group, a mercaptonaphthyl group, an aminonaphthyl group, a carbamylnaphthyl group, a sulfonamidonaphthyl group, a sulfamylnaphthyl group, a nitronaphthyl group, etc.) etc., and a heterocyclic group, preferably containing from five to six atoms, and preferably containing hereto atoms, such as nitrogen, sulfur, oxygen and selenium, such as, for example, a thiazolyl group, a benzothiazolyl group, an oxazolyl group, a benzoxazolyl group, a selenazolyl group, a benzoselenazolyl group, a benzimidazolyl group, a triazinyl group, a pyrimidinyl group, a pyridyl group, a quinolyl group, a thienyl group, etc.;  $R_2$  represents any of the groups represented by  $R_1$  and, in addition, represents an alkyl group (e.g., methyl, butyl, hexyl, dodecyl, mercaptomethyl, mercaptoethyl, etc.) etc., hydrogen, hydroxyl, carboxyl, a salt of a carboxyl group (e.g., an alkali metal salt or ammonium salt), a carboxy ester group (e.g., methoxycarbonyl, ethoxycarbonyl, phenoxy carbonyl, etc.), an amino group (e.g., amino, ethylamino, dimethylamino, anilino, etc.), a carbamyl group (e.g., carbamyl, ethylcarbamyl, dimethylcarbamyl, phenylcarbamyl, etc.), sulfo, a salt of a sulfo group (e.g., an alkali metal salt), a sulfamido group (e.g., methylsulfonamido, butylsulfonamido, phenylsulfonamido, etc.), a sulfamyl group (e.g., sulfamyl, methylsulfamyl, butylsulfamyl, phenylsulfamyl, etc.), the mercapto group, the nitro group, or any other substituent cited as being present in this position of the formazan or the tetrazolium salt in Chem. Rev. 55, 355-483 (1955); and the substituents  $R_1$  and  $R_3$  can advantageously contain an electron-sharing group capable of forming metal chelates or complexes, such as primary, secondary and tertiary amino, substituted amino, oxime, thioether, keto, thioketo, hydroxyl, mercapto, carboxyl, carboxyl, sulfo, phospho, alkoxy groups or complexes;  $X^\ominus$  represents an anion (e.g., chloride, iodide, bromide, sulfate, paratoluenesulfonate, methylsulfate, ethylsulfate, nitrate, acetate, perchlorate, perborate, sulfite, hydroxide, carbonate, etc.); D represents a divalent aromatic group (e.g., a phenylene, diphenylene, naphthalene, phenylmethylphenyl, etc.); and E represents a divalent group such as an alkylene group (e.g., methylene, ethylene, propylene, butylene, etc.), an arylene group (e.g., phenylene, naphthalene, diphenylene, etc.), an arylene alkylene group, for example, a phenylene alkylene group (e.g., phenylene methylene, phenylene butylene, phenylene hexylene, etc.), a naphthylene alkylene group (e.g., naphthylene methylene, naphthylene butylene, naphthylene propylene, etc.), etc;  $n$  represents an integer of from 1 to 5.

Tetrazolium salts used to advantage according to our invention include the following representative compounds:

|                                                                           |    |                                                                                                         |
|---------------------------------------------------------------------------|----|---------------------------------------------------------------------------------------------------------|
| 2,3,5-triphenyl-2H-tetrazolium chloride                                   | 55 | 3-(p-sulfamylphenyl)-3-phenyl-5-propyl-2H-tetrazolium chloride                                          |
| 2,3,5-tri(p-carboxyethylphenyl)-2H-tetrazolium bromide                    |    | 2,3-diphenyl-5-isobutyl-2H-tetrazolium chloride                                                         |
| 2-(benzothiazol-2-yl)-3-phenyl-5-(o-chlorophenyl)-2H-tetrazolium chloride | 60 | 2,3-diphenyl-5-n-hexyl-2H-tetrazolium chloride                                                          |
| 2-(4,5-dimethylthiazol-2-yl)-3,5-diphenyl-2H-tetrazolium bromide          |    | 2-phenyl-3-(p-sulfamylphenyl)-5-hexyl-2H-tetrazolium chloride                                           |
| 2,3-diphenyl-2H-tetrazolium chloride                                      | 65 | 2,3-diphenyl-5-dodecyl-2H-tetrazolium chloride                                                          |
| 2,3-diphenyl-2H-tetrazolium iodide                                        |    | 2,3-diphenyl-5-hydroxy-2H-tetrazolium betaine                                                           |
| 2,3-diphenyl-5-methyl-2H-tetrazolium chloride                             |    | 2,3-diphenyl-5-mercaptop-2H-tetrazolium betaine                                                         |
| 2,3-diphenyl-5-methyl-2H-tetrazolium bromide                              | 70 | 5-amino-2,3-diphenyl-2H-tetrazolium chloride                                                            |
| 3-(p-hydroxyphenyl)-5-methyl-2-phenyl-2H-tetrazolium chloride             |    | 5-benzamido-2,3-diphenyl-2H-tetrazolium chloride                                                        |
| 3-(o-carboxyphenyl)-5-methyl-2-phenyl-2H-tetrazolium chloride             |    | 5-benzamido-2,3-diphenyl-2H-tetrazolium betaine                                                         |
| 3-(p-carboxyphenyl)-5-methyl-2-phenyl-2H-tetrazolium chloride             |    | 5-cyano-2,3-diphenyl-2H-tetrazolium chloride                                                            |
| 3-(p-sulfamylphenyl)-5-methyl-2-phenyl-2H-tetrazolium chloride            | 75 | 5-carboxy-2,3-diphenyl-2H-tetrazolium betaine                                                           |
| 2,3-diphenyl-5-ethyl-2H-tetrazolium chloride                              |    | 5-carboxy-2,3-diphenyl-2H-tetrazolium chloride                                                          |
|                                                                           |    | 5-carboxy-2,3-diphenyl-2H-tetrazolium nitrate                                                           |
|                                                                           |    | 3-(benzothiazol-2-yl)-5-(4-hexoxyphenyl)-2-(3-sulfophenyl)-2H-tetrazolium                               |
|                                                                           |    | 2-benzothiazol-2-yl)-3-phenyl-5-[4-(3,5-disulfobenzamido)phenyl]-2H-tetrazolium bromide (disodium salt) |
|                                                                           |    | 2-(benzothiazol-2-yl)-5-(2-chlorophenyl)-3-(4-nitrophenyl)-2H-tetrazolium bromide                       |
|                                                                           |    | 2-(benzothiazol-2-yl)-5-phenyl-3-(4-tolyl)-2H-tetrazolium bromide                                       |
|                                                                           |    | 2-(benzothiazol-2-yl)-3-(4-chlorophenyl)-5-phenyl-2H-tetrazolium bromide                                |
|                                                                           |    | 2-(benzothiazol-2-yl)-5-(4-chlorophenyl)-3-(4-nitrophenyl)-2H-tetrazolium bromide                       |
|                                                                           |    | 5-ethoxycarbonyl-2,3-diphenyl-2H-tetrazolium chloride                                                   |
|                                                                           |    | 5-ethoxycarbonyl-2,3-di(3-nitrophenyl)-2H-tetrazolium chloride                                          |
|                                                                           |    | 5-carboxy-2,3-di(p-hydroxyphenyl)-2H-tetrazolium betaine                                                |
|                                                                           |    | 5-carboxy-2,3-di(p-ethoxyphenyl)-2H-tetrazolium chloride                                                |
|                                                                           |    | 2,3-di(p-ethoxyphenyl)-5-ethoxycarbonyl-2H-tetrazolium chloride                                         |
|                                                                           |    | 5-acetyl-2,3-diphenyl-2H-tetrazolium chloride                                                           |
|                                                                           |    | 5-benzoyl-2,3-diphenyl-2H-tetrazolium chloride                                                          |
|                                                                           |    | 2,5-diphenyl-3-(p-tolyl)-2H-tetrazolium bromide                                                         |
|                                                                           |    | 2,5-diphenyl-3-(p-isopropylphenyl)-2H-tetrazolium bromide                                               |
|                                                                           |    | 2,5-diphenyl-3-(p-n-dodecylphenyl)-2H-tetrazolium iodide                                                |
|                                                                           |    | 2,5-diphenyl-3-(p-diphenyl)-2H-tetrazolium chloride                                                     |
|                                                                           |    | 2,3-diphenyl-5-(p-diphenyl)-2H-tetrazolium chloride                                                     |
|                                                                           |    | 2,5-diphenyl-3-(p-chlorophenyl)-2H-tetrazolium iodide                                                   |
|                                                                           |    | 2,5-diphenyl-3-(iodophenyl)-2H-tetrazolium chloride                                                     |
|                                                                           |    | 3,5-di(p-bromophenyl)-2-phenyl-2H-tetrazolium chloride                                                  |
|                                                                           |    | 5-(p-bromophenyl)-2-phenyl-3-(2,4,6-tribromophenyl)-2H-tetrazolium bromide                              |
|                                                                           |    | 3-(p-iodophenyl)-2-(p-nitrophenyl)-5-phenyl-2H-tetrazolium chloride                                     |
|                                                                           |    | 3-(p-hydroxyphenyl)-5-(p-nitrophenyl)-2-phenyl-2H-tetrazolium chloride                                  |
|                                                                           |    | 5-(3,4-dimethoxyphenyl)-3-methoxyphenyl-2-phenyl-2H-tetrazolium iodide                                  |
|                                                                           |    | 5-(3-methoxyphenyl)-3-(3-trifluoromethylphenyl)-2-phenyl-2H-tetrazolium acetate                         |
|                                                                           |    | 2-(3-carboxyphenyl)-3,5-diphenyl-2H-tetrazolium iodide                                                  |
|                                                                           |    | 5-(4-cyanophenyl)-2,3-diphenyl-2H-tetrazolium chloride                                                  |
|                                                                           |    | 2,3-diphenyl-5-sulfophenyl-2H-tetrazolium betaine                                                       |
|                                                                           |    | 3-(p-aminophenyl)-2,5-diphenyl-2H-tetrazolium chloride                                                  |
|                                                                           |    | 3-(p-acetamidophenyl)-2,5-diphenyl-2H-tetrazolium chloride                                              |
|                                                                           |    | 5-(4-aminophenyl)-2,3-diphenyl-2H-tetrazolium chloride                                                  |
|                                                                           |    | 5-acetyl-2,3-diphenyl-2H-tetrazolium chloride                                                           |
|                                                                           |    | 2,3-diphenyl-5-(4-phenylsulfamylphenyl)-2H-tetrazolium hydroxide                                        |
|                                                                           |    | 3-(4-amino-3-chlorophenyl)-2,5-diphenyl-2H-tetrazolium chloride                                         |
|                                                                           |    | 3-(4-amino-2-nitrophenyl)-2,5-diphenyl-2H-tetrazolium chloride                                          |
|                                                                           |    | 3-(4-amino-3-hydroxyphenyl)-2,5-diphenyl-2H-tetrazolium chloride                                        |
|                                                                           |    | 2,5-diphenyl-3-(4-octadecylaminophenyl)-2H-tetrazolium chloride                                         |

3-amino-2,5-diphenyl-2H-tetrazolium chloride  
 2,5-diphenyl-3-(4-N-trimethylammoniumphenyl)-2H-tetrazolium methylsulfate  
 3-(2-benzyloxyphenyl)-5-(4-N-trimethylammoniumphenyl)-2-phenyl-2H-tetrazolium chloride  
 5-(fur-2-yl)-2,3-diphenyl-2H-tetrazolium chloride  
 5-(fur-2-yl)-3-(4-chlorophenyl)-2-quinol-2-yl)-2H-tetrazolium acetate  
 5-(thien-2-yl)-2,3-diphenyl-2H-tetrazolium chloride  
 2,3-diphenyl-5-(pyrid-2-yl)-2H-tetrazolium bromide  
 2,3-diphenyl-5-(pyrid-4-yl)-2H-tetrazolium chloride  
 2,5-diphenyl-3-(pyrid-3-yl)-2H-tetrazolium chloride  
 2-(4-chlorophenyl)-3-(2-chlorophenyl)-5-(pyrid-2-yl)-2H-tetrazolium acetate  
 2,3-diphenyl-5-(quinol-2-yl)-2H-tetrazolium bromide  
 2,3-diphenyl-5-(benzoxazol-2-yl)-2H-tetrazolium chloride  
 2,3-di(4-bromophenyl)-5-(benzothiazol-2-yl)-2H-tetrazolium chloride  
 2,3-diphenyl-5-(2-phenyltriazol-5-yl)-2H-tetrazolium chloride  
 2,3-diphenyl-5-nitro-2H-tetrazolium chloride  
 2,3-diphenyl-5-sulfo-2H-tetrazolium chloride  
 2,3-diphenyl-5-sulfonamido-2H-tetrazolium chloride  
 2,2',3,3'-tetraphenyl-5,5'-diethylene di-(2H-tetrazolium chloride)  
 2,2',3,3'-tetraphenyl-5,5'-di-1,6-hexylene di-(2H-tetrazolium chloride)  
 2,2',3,3'-tetraphenyl-5,5'-di-p-phenylene di-(2H-tetrazolium chloride)  
 5,5'-dimethyl-3,3'-diphenyl-2,2'-di-p-diphenylene di-(2H-tetrazolium chloride)  
 3,3',5,5'-tetraphenyl-2,2'-di-p-(3,3'-dimethyl-diphenylene) di-(2H-tetrazolium chloride)  
 3,3'-diphenyl-5,5'-di(thien-2-yl)-2,2'-di-p-(3,3'-di-methoxydiphenylene) di-(2H-tetrazolium chloride)  
 3,3',5,5'-tetraphenyl-2,2'-syn-p-phenylthiourea di-(2H-tetrazolium chloride)  
 3,3',5,5'-tetraphenyl-2,2'-syn-p-phenyl sulfoxide di-(2H-tetrazolium chloride)  
 2,2',3,3'-tetraphenyl-5,5'-p-phenylene ethylene di-(2H-tetrazolium chloride)  
 2-(benzothiazol-2-yl)-5-(4-acetamidophenyl)-3-(4-phenylazophenyl)-2H-tetrazolium bromide  
 2-(benzothiazol-2-yl)-3-(4-methoxyphenyl)-5-phenyl-2H-tetrazolium bromide  
 2-(4,5-dimethylthiazol-2-yl)-3,5-diphenyl-2H-tetrazolium bromide  
 2-(4-chlorophenyl)-3-(2-chlorophenyl)-5-(pyrid-2-yl)-2H-tetrazolium acetato  
 2,3-diphenyl-5-(quinol-2-yl)-2H-tetrazolium bromide  
 2-(benzimidazol-2-yl)-5-(2-chlorophenyl)-3-phenyl-2H-tetrazolium chloride  
 5-(2-chlorophenyl)-3-phenyl-2-(thien-2-yl)-2H-tetrazolium chloride  
 3,5-diphenyl-2-(pyrid-2-yl)-2H-tetrazolium chloride  
 3,5-diphenyl-2-(triazin-2-yl)-2H-tetrazolium chloride

These tetrazolium salts are well known in the art, most of them having been described in literature references such as Chemical Revue 55, published bimonthly for the American Chemical Society by the Williams and Wilkins Co., Baltimore, 1955. Any tetrazolium salts that are not shown specifically in the prior art are advantageously prepared by methods well known in the art.

When aqueous solutions of our T-salts, brought into contact with metal images of palladium or any metal more easily oxidized (i.e., has a standard oxidation potential more positive than  $-0.98$  volt) (e.g., silver, nickel, copper, iron, palladium, zinc, lead, tin, etc.), the metal is oxidized to its ion and the T-salt is reduced to produce the corresponding formazan dye. The following equation shows a typical reaction.



Any ligand that is a silver complexing agent is advantageously used that produces a silver ion complex with a cumulative equilibrium constant  $\beta_2$ , i.e.,

$$\beta_2 = \frac{\text{(concentration of silver ion complex)}}{\text{(concentration of silver ion)} \times \text{(concentration of complexing agent)}^2}$$

that is smaller than the  $\beta_2$  for the silver complexed with cyanide ion in a given solvent system at about 20° C. The  $\beta_2$  constants used herein are measured with a silver electrode in contact with a solution (at 20° C.) of the complexing agent to which is being added silver ions as is described in "Stability Constants of Metal-Ion Complexes," in Special Publications No. 17, published in London by The Chemical Society in 1964. This reference cites numerous cumulative equilibrium constants that are measured in an aqueous medium, except when the complexing agent doesn't have the desired solubility in water, then a solvent or solvent mixture is used in which both complexing agent and complex are soluble, the tests being the same as in other instances where the complexing agent is water-soluble. Metal images other than silver are also advantageously converted for formazan dye images. Preferably, a silver complexing agent is employed that produces with silver a complex with a  $\beta_2$  value that is less than about 10<sup>17</sup> which is about 10<sup>3</sup> times smaller than the  $\beta_2$  of 10<sup>20</sup> for silver ions complexed with cyanide ions. By a diffusible metal complex, we mean a metal complex that in water solution can pass freely through photographic silver halide emulsion layers. Included among the ligands used to advantage are the following typical examples: water-soluble thiosulfates (e.g., sodium thiosulfate, potassium thiosulfate, ammonium thiosulfate, etc.), thiourea, ethylenethiourea, a water-soluble thiocyanate (e.g., sodium thiocyanate, potassium thiocyanate, ammonium thiocyanate), a water-soluble sulfur containing dibasic acid. Water-soluble diols used to advantage include those having the formula:



wherein  $p$  is an integer of from 2 to 13; the Z's represent oxygen or sulfur atoms such that at least one-third of the Z atoms are sulfur and there are at least two consecutive Z's in the structure of the compound which are sulfur atoms. The diols advantageously used are also included in compounds having the formula:



wherein X and  $X^1$  represent oxygen or sulfur, such that when  
 60 X represents oxygen,  $X^1$  represents sulfur and when X  
 represents sulfur,  $X^1$  represents oxygen; c, d, e, f and g each  
 represent an integer of from 1 to 15, such that the sum of  
 $c+d+e+f+g$  represents an integer of from 6 to 19, and such  
 that at least one third of the total of all the X's plus all the  $X^1$ 's  
 65 represent sulfur atoms and at least two consecutive X's and/or  
 $X^1$ 's in the structure of the compound are sulfur atoms.

Typical diols include the following:

- 70 1. 3,6-Dithia-1,8-octanediol  

$$\text{HOCH}_2\text{CH}_2\text{SCH}_2\text{CH}_2\text{SCH}_2\text{CH}_2\text{OH}$$

2. 3,6,9-Trithia-1,11-undecanediol  

$$\text{HOCH}_2\text{CH}_2\text{SCH}_2\text{CH}_2\text{SCH}_2\text{CH}_2\text{SCH}_2\text{CH}_2\text{OH}$$

3. 3,6,9,12-Tetrathia-1,14-tetradecanediol  

$$\text{HO}(\text{CH}_2\text{CH}_2\text{S})_4\text{CH}_2\text{CH}_2\text{OH}$$

75 4. 9-Oxa-3,6,9,12, 15-tetrathia-1,17-heptadecanediol

HO(CH<sub>2</sub>CH<sub>2</sub>S)<sub>2</sub>CH<sub>2</sub>CH<sub>2</sub>O(CH<sub>2</sub>CH<sub>2</sub>S)<sub>2</sub>CH<sub>2</sub>CH<sub>2</sub>OH  
 5. 9,12-Dioxa-3,6,15,18-tetrathia-1,20-eicosanediol  
 HO(CH<sub>2</sub>CH<sub>2</sub>S)<sub>2</sub>(CH<sub>2</sub>CH<sub>2</sub>O<sub>5</sub>(CH<sub>2</sub>CH<sub>2</sub>S)<sub>2</sub>CH<sub>2</sub>OH  
 6. 3,6-Dioxa-9,12-dithia-1,14-tetradecanediol  
 HO(CH<sub>2</sub>CH<sub>2</sub>O)<sub>2</sub>(CH<sub>2</sub>CH<sub>2</sub>S)<sub>2</sub>CH<sub>2</sub>CH<sub>2</sub>OH  
 7. 3,12-Dioxa-6,9-dithia-1,14-tetradecanediol  
 HOCH<sub>2</sub>CH<sub>2</sub>O(CH<sub>2</sub>CH<sub>2</sub>S)<sub>2</sub>CH<sub>2</sub>CH<sub>2</sub>OCH<sub>2</sub>CH<sub>2</sub>OH  
 8. 3,18-Dioxa-6,9,12,15-tetrathia-1,20-eicosanediol  
 HOCH<sub>2</sub>CH<sub>2</sub>O(CH<sub>2</sub>CH<sub>2</sub>S)<sub>4</sub>CH<sub>2</sub>CH<sub>2</sub>OCH<sub>2</sub>CH<sub>2</sub>OH  
 9. 12,18-Dioxa-3,6,9,15,21,24,27-heptathia-1,29-  
 nonacosanediol  
 HO(CH<sub>2</sub>CH<sub>2</sub>S)<sub>3</sub>CH<sub>2</sub>CH<sub>2</sub>OCH<sub>2</sub>CH<sub>2</sub>SCH<sub>2</sub>CH<sub>2</sub>O(CH<sub>2</sub>CH<sub>2</sub>-  
 S)<sub>3</sub>CH<sub>2</sub>CH<sub>2</sub>OH  
 10. 6,9,15,18-Tetrathia-3,12,21-trioxa-1,23-tricosanediol  
 HOCH<sub>2</sub>CH<sub>2</sub>O(CH<sub>2</sub>CH<sub>2</sub>S)<sub>2</sub>CH<sub>2</sub>CH<sub>2</sub>O(CH<sub>2</sub>CH<sub>2</sub>S)<sub>2</sub>CH<sub>2</sub>CH<sub>2</sub>-  
 OCH<sub>2</sub>CH<sub>2</sub><sup>OH</sup>

Water-soluble sulfur containing dibasic acids used to advantage include those having the formula:



in which  $q$  represents an integer of from 1 to, and including, 3 and the alkali metal and ammonium salts of said acids. Typical illustrative examples include:

ethylene-bis-thioglycolic acid  
 HOOCCH<sub>2</sub>SCH<sub>2</sub>CH<sub>2</sub>SCH<sub>2</sub>COOH  
 3,6,9-trithiahendecanedioic acid  
 HOOCCH<sub>2</sub>(SCH<sub>2</sub>CH<sub>2</sub>)<sub>2</sub>SCH<sub>2</sub>COOH  
 3,6,9,12-tetrathiatetradecanedioic acid  
 HOOCCH<sub>2</sub>(SCH<sub>2</sub>CH<sub>2</sub>)<sub>3</sub>SCH<sub>2</sub>COOH  
 ethylene-bis-thioglycolic acid disodium salt  
 ethylene-bis-thioglycolic acid dipotassium salt  
 ethylene-bis-thioglycolic acid diammonium salt  
 3,6,9-trithiahendecanedioic acid disodium salt  
 3,6,9,12-tetrathiatetradecanedioic acid disodium salt

The concentration of the T-salt and the ligand in our compositions can be varied considerably, with an operable range of concentrations extending from the solubility limit of the T-salt and the solubility limit of the ligand down to a minimum concentration where the overall reaction potential for the specific T-salt, ligand and specific metal image just remains positive, usually above +0.01 volt. The operable concentration ranges and the preferred concentration ranges are readily determined by methods well known in the art and need not be discussed further.

The metal images that are advantageously treated with our T-salt ligand compositions are produced by any of the conventional image-forming methods and especially by photographic methods, using chemical developing-out materials, physical developing-out materials, etc. The metal image is advantageously made up of minute particles of metal in a binder, e.g., a hydrophilic colloid such as, gelatin or gelatin substitute, or made of a solid, continuous surface of metal.

The following examples are included for a further understanding of our invention:

Example 1 - Conversion of a Silver Image to a Formazan Dye Image

A sample of a supported negative type, developing-out, single-layer fine-grain gelatinous silver chlorobromide emulsion, having been exposed to a graduated-density test object, black-and-white developed in a conventional aqueous alkaline p-methylaminophenol and hydroquinone developer solution, fixed in a conventional alkali metal thiosulfate fixing bath, washed and dried, is treated for 4 minutes at 75° F. in Solution A (see composition below), washed and dried. Solution A is made by dissolving the following composition:

|                                                               |        |
|---------------------------------------------------------------|--------|
| Ma <sub>2</sub> HPO <sub>4</sub>                              | 10 g.  |
| (NH <sub>4</sub> ) <sub>2</sub> S <sub>2</sub> O <sub>8</sub> | 200 g. |
| Thiourea                                                      | 10 g.  |
| 2,1,5-triphenyl 2H-tetrazolium                                |        |
| chloride                                                      | 10 g.  |

in 600 ml. of water, then bringing the total volume to 1 liter. Solution A has a pH of 7. Sensitometric curves of the images in the sample before and after treatment in Solution A show a

pronounced increase in image density obtained by the conversion of a metallic silver image to formazan dye by a solution according to our invention. The  $\lambda_{\text{max}}$  of the formazan dye is 490 m $\mu$ .

5 Example 2 - pH-Independence and Solution Stability

Three samples of a negative type developing-out fine-grain gelatinous silver bromoiodide emulsion coated film, each having been flash-exposed, black-and-white developed to a neutral density of 0.7 in a conventional black-and-white developer as used in Example 1, fixed in a conventional alkali metal thiosulfate fixing bath, washed and dried, are treated for 2 minutes at 75° F. in portions of Solution B (see formula below) whose pH values are 4.3, 6.1, and 10.0, respectively.

10 15 The samples are subsequently washed and dried. The dye densities in the three samples are essentially the same, as is shown in Table 1. The solutions are kept for 96 hours at room temperature and then used to repeat the above procedure with three similar samples. Essentially the same dye densities are obtained. Solution B is made by dissolving a composition containing 1 of 2,3,5-triphenyl-2H-tetrazolium chloride and 10 g. of ammonium thiosulfate in water to make 100 ml. of solution.

20

Table 1

25

| Sample No. | Density at 500 m $\mu$ | pH of solution B           |
|------------|------------------------|----------------------------|
| 30 Check   | 0.7                    | no treatment in Solution B |
| 1          | 0.95                   | 4.3                        |
| 2          | 0.93                   | 6.1                        |
| 3          | 0.95                   | 10.0                       |

The data in Table 1 indicate that the conversion of a metal image to a formazan dye image by a procedure according to our invention is effectively accomplished over a wide range of pH conditions.

40 Example 3 - Spectral Distribution of the Light Absorption of Image Formazan Dye vs. Image Silver

A sample of the silver halide emulsion coated film described in Example 2 is flash-exposed, black-and-white developed, fixed, washed and dried as described in Example 2. The density of the silver image to red, green and blue light is recorded under "Untreated Area" in Table 2. Upon treatment of the sample for 60 minutes at 75° F. in Solution C (see composition below), the initial silver image is converted to a brown formazan dye image whose density to red, green and blue light is recorded under "Treated Area" in Table 2. Solution C is made by dissolving a composition containing 1 g. of 2-(benzothiazol-2-yl)-3-phenyl-5-(o-chlorophenyl)-2H-tetrazolium bromide and 10 g. of ammonium thiosulfate in water to make 100 ml. of solution having a pH of 10.

55

Table 2

|                   | Red  | Green | Blue |
|-------------------|------|-------|------|
| 60 Untreated area | 0.45 | 0.54  | 0.67 |
| Treated area      | 0.42 | 0.65  | 0.94 |

The above data illustrate that a silver image of a given spectral density is effectively converted to a formazan dye image having an overall higher spectral density.

65 Example 4 - Mixtures of T-salts Are Used To Adjust Color Of Dye Image

Four samples of the silver halide emulsion coated film described in Example 2, having been flash-exposed, black-and-white developed, fixed, washed and dried as described in Example 2, are treated for 2 minutes at 75° F. in Solution B (pH 8, described in Example 2) and in Solution D (described below) and in mixtures thereof as shown in Table 3. The obtained formazan dye images range in color from red to blue.

Their spectral absorption to the red, green and blue regions of the visible spectrum is illustrated in Table 3. Solution D is made by dissolving a composition containing 1 g. of 2-(4,5-dimethylthiazol-2-yl)-3,5-diphenyl-2H-tetrazolium bromide and 10 g. of ammonium thiosulfate in water to make 100 ml. of solution having a pH of 8.0.

Table 3

|                                | Red  | Green | Blue |
|--------------------------------|------|-------|------|
| Solution B                     | 0.4  | 0.88  | 0.64 |
| Solution D                     | 0.66 | 1.06  | 0.66 |
| 100 ml. soln. B/20 ml. soln. D | 0.64 | 0.94  | 0.60 |
| 100 ml. soln. B/30 ml. soln. D | 0.76 | 0.98  | 0.63 |

**Example 5 - Silver Images In A Variety Of Photographic Materials Are Convertible To Formazan Dye Images**

Black-and-white processed (i.e., developed, fixed, washed and dried as described in Example 1) samples of several types of negative type, developing-out photographic materials are treated from 1 to 16 minutes in portions of Solution B (see Example 2) ranging in pH from 6 to 12 to produce formazan dye images essentially as described in the preceding examples. The photographic materials include:

1. A coarse-grain gelatinous silver bromoiodide X-ray film
2. A fine-grain gelatinous silver bromoiodide film
3. Supported gelatinous layers containing Carey Lea silver, and
4. Several fine-grain gelatinous silver bromoiodide emulsion coated Micro-File films (Kodak Trademark)

The results show our Solution B is an active Blix for removing silver from photographic layers. The density and spectral absorption characteristics of the formazan dyes to which the silver is converted during the above treatments in Solution B are similar to the values cited in the preceding examples.

**Example 6 - Electron Transfer Catalyst Accelerates Rate Of Dye Formation**

Two black-and-white processed (i.e., developed, fixed, washed and dried as described in Example 1) samples of the X-ray film described in Example 5 are treated at 75° F. and pH 10.0 for 2 and 10 minutes, respectively, in Solution B (see Example 2). Two other samples are similarly treated, except that 2 g. of the electron transfer agent N,N,N',N'-tetramethyl-p-phenylenediamine hydrochloride, are added to a 100-ml. portion of Solution B. The density of the formazan dye images in the two samples treated in the presence of the electron transfer agent is higher than the density in the samples treated in Solution B not containing the agent. This observation illustrated by the data in Table 4.

Table 4

|                                | Red tg | Green | Blue |
|--------------------------------|--------|-------|------|
| Solution B, 2 min.             | 0.64   | 0.61  | 0.54 |
| Solution B plus agent, 2 min.  | 0.79   | 0.80  | 0.66 |
| Solution B, 10 min.            | 0.71   | 0.79  | 0.70 |
| Solution B plus agent, 10 min. | 0.84   | 1.02  | 0.82 |

**Example 7 - Certain Organic Solvents Increase Rate Of Dye Formation**

Two black-and-white processed (i.e., developed, fixed, washed and dried as described in Example 1) samples of a negative type, developing out fine-grain gelatinous silver chlorobromide emulsion Micro-File films are treated at 115°

F. and pH 7.0 in Solutions E and F (compositions below), respectively, for 0, 15, 30, 60 and 120 seconds. The data recorded in Table 5 indicate that benzyl alcohol increases the rate of the conversion from image silver to formazan dye. 5 Solution E is made by dissolving a composition containing 1 g. of 2,3,5-triphenyl-2H-tetrazolium chloride, 20 g. of ammonium thiosulfate and 0.1 g. of thiourea in water to make 100 ml. of solution. Solution F is made by adding 0.4 ml. of benzyl alcohol to 100 ml. of Solution E.

Table 5

|            | mg. of AG/ft. <sup>2</sup> Remaining in Film after Treatment |         |         |         |          |
|------------|--------------------------------------------------------------|---------|---------|---------|----------|
|            | 0 sec.                                                       | 15 sec. | 30 sec. | 60 sec. | 120 sec. |
| Solution E | 180                                                          | 30      |         | 17      | 15       |
| Solution F | 180                                                          | 46      | 14      | 10      | 8        |

**Example 8 - Mixtures of Metal Complexing Agents Increase The Rate Of Dye Formation**

A first sample of a sensitometrically exposed, developed, fixed, washed and dried, negative type, developing-out, fine-grain gelatinous silver bromoiodide emulsion coated film is treated at 75° F. for 2 minutes in Solution G (see composition below). Solution G is made by dissolving the following composition:

|    |                                                               |         |
|----|---------------------------------------------------------------|---------|
| 30 | 2,3,5-tri phenyl-2H-tetrazolium chloride                      | 1 g.    |
|    | (NH <sub>4</sub> ) <sub>2</sub> S <sub>2</sub> O <sub>8</sub> | 10 g.   |
|    | Disodium phosphate                                            | 1 g.    |
|    | Benzyl alcohol                                                | 0.8 ml. |
|    | Ethylene thiourea                                             | 0.01 g. |

35 in water to make 100 ml. of solution. A second and a third sample are treated similarly except that Solution G contained 0.1 g. and 1.0 g. of ethylene thiourea, respectively. The increase in the rate of conversion of silver to formazan dye with increased concentration of a second silver complexing agent, such as ethylene thiourea, is illustrated in Table 6.

Table 6

| 45 | Amount of Ethylene thiourea in 100 ml. solution | Formazan dye density at step  |      |        |
|----|-------------------------------------------------|-------------------------------|------|--------|
|    |                                                 | Number of sensitometric strip | 17   | 15     |
| 50 | First                                           | 0.01 g.                       | 0.28 | 0.82   |
|    | Second                                          | 0.1 g.                        | 0.31 | 0.97   |
|    | Third                                           | 1.0 g.                        | 0.40 | 1.18   |
|    |                                                 |                               |      | 2.94 v |

**Example 9 - Rate Of Removal Of Silver From A Variety Of Photographic Materials Increases With Increased Temperature**

A selectively balanced Blix composition according to our invention effectively removes the image silver from various types of processed photographic materials. The rate of silver removal increases with increased temperature. Silver images in several exposed, developed, fixed, washed and dried coarse-grain gelatinous silver halide X-ray films and a fine-grain gelatinous silver halide film are treated for various times at temperatures of 75° F., 100° F. and 125° F. in portions of Solution B (see Example 2). These films are coated with negative type, developing out gelatinous-silver bromoiodide emulsions. The effect of temperature on the rate and amount of silver removal is illustrated by the data recorded in Table 7.

TABLE 7

| Photogr. material | Temp., °F. | Mg. Ag/ft. <sup>2</sup> remaining in film after treatment in Solution B for— |        |        |        |         |
|-------------------|------------|------------------------------------------------------------------------------|--------|--------|--------|---------|
|                   |            | 0 min.                                                                       | 1 min. | 4 min. | 8 min. | 16 min. |
| An X-ray film     | 75         | 80                                                                           | 60     | 36     | 26     | 20      |
|                   | 100        | 80                                                                           | 34     | 20     | 14     | 12      |
|                   | 125        | 80                                                                           | 36     | 24     | 10     | 0       |

TABLE 7

| Photogr. material           | Temp.<br>°F. | Mg. Ag/ft. <sup>2</sup> remaining in film after treatment in<br>Solution B for— |        |        |        |         |
|-----------------------------|--------------|---------------------------------------------------------------------------------|--------|--------|--------|---------|
|                             |              | 0 min.                                                                          | 1 min. | 4 min. | 8 min. | 16 min. |
| A black-and-white film..... | 75           | 205                                                                             | 275    | 220    | 170    | 90      |
|                             | 100          | 205                                                                             | 280    | 134    | 104    | 54      |
|                             | 125          | 295                                                                             | 216    | 40     | 30     | 18      |
| A second X-ray film.....    | 75           | 112                                                                             | 102    | 66     | 52     | 50      |
|                             | 100          | 112                                                                             | 76     | 60     | 50     | 2       |
|                             | 125          | 112                                                                             | 54     | 10     | 8      | 0       |
| A third X-ray film.....     | 75           | 88                                                                              | 68     | 38     | 34     | 30      |
|                             | 100          | 88                                                                              | 34     | 32     | 30     | 24      |
|                             | 125          | 88                                                                              | 34     | 24     | 10     | 0       |

Similar results are obtained when a developed (but unbleached and unfixed) multicolor, multilayer color film is blixed with our composition.

Example 10 - Formazan Dye Images Are Sharper Than the Initial Silver Images From Which They Are Derived

A sensitometrically exposed negative type, developing-out coarse-grain gelatinous silver bromoiodide X-ray film is developed, fixed washed and dried as described in Example 1. One sample of this processed film is used as a control: a second sample is treated for 4 minutes in Solution G (see Example 8) and a third sample is treated for 8 minutes in Solution G. The densities of the resulting images to blue light in each of the processed film samples are measured with a densitometer. The density data for the first, ninth and 17th steps of the sensitometric images are listed in Table 8 below:

Table 8

| Film Sample | Treatment Time<br>in Solution G | Density to Blue Light at<br>Step 17 | Step 9 | Step 1 |
|-------------|---------------------------------|-------------------------------------|--------|--------|
| 1           | 0 (control)                     | 0.27                                | 1.28   | 1.60   |
| 2           | 4 min.                          | 0.34                                | 1.40   | 1.80   |
| 3           | 8 min.                          | 0.45                                | 2.00   | 2.64   |

These data show the increase in image density produced by treatment of film samples with Solution G. X-ray line exposures made on Film Samples 4, 5 and 6 as described in Rev. of Scientific Instruments, 38, No. 11 pages 1,619-1,622, Nov. 19, 1967 are processed as described for Samples 1, 2 and 3, respectively, in this example. Microdensitometric traces of the resulting images indicate the formazan dye images in Film Samples 5 and 6 are sharper than the silver image in Sample 4. Example 11 - Silver Images In Direct Reversal Emulsions Are Effectively Converted to Formazan Dye Images

Five samples of a coating of a direct-positive type, developing-out, gelatinous silver chlorobromoiodide emulsion are exposed to a graduated density test object and black-and-white developed to a direct positive image reproduction.  $\rho_{max}$ ,  $\rho_{min}$ , and gamma of the sensitometric curve (i.e., a curve of image density vs. exposure) representing the image in one of the samples are recorded in Table 9. The remaining four samples are subsequently treated at 75° F. for 1, 2, 4 and 8 minutes, respectively, in Solution H (see composition below). Solution H is made by dissolving the following composition:

|                                                               |         |
|---------------------------------------------------------------|---------|
| Na <sub>2</sub> HPO <sub>4</sub>                              | 1 g.    |
| (NH <sub>4</sub> ) <sub>2</sub> S <sub>2</sub> O <sub>8</sub> | 20 g.   |
| Thiourea                                                      | 1 g.    |
| Benzyl alcohol                                                | 0.4 ml. |
| 2,3,5-triphenyl-2H-tetrazolium chloride                       | 1 g.    |

in water to make 100 ml. of solution of pH 7.0.  $\rho_{max}$ ,  $\rho_{min}$ , and gamma of the sensitometric curves (read through a green filter) representing the corresponding formazan dye images are recorded in Table 9.

TABLE 9

|                    | time in<br>Soln. H | $\rho_{max}$ | $\rho_{min}$ | Gamma |
|--------------------|--------------------|--------------|--------------|-------|
| Sample 1 (control) | 0                  | 1.35         | 0.1          | 0.96  |
| Sample 2           | 1 min.             | 2.36         | 0.12         | 1.82  |
| Sample 3           | 2 min.             | 3.00         | 0.16         | 2.3   |
| Sample 4           | 4 min.             | 3.20         | 0.16         | 2.6   |
| Sample 5           | 8 min.             | 3.36         | 0.18         | 2.6+  |

Example 12 - Conversion of Nickel and Copper Images To Formazan Dye Images

30 A first sample of a nickel image reproduction prepared by physically developing an exposed photosensitive material of the type containing a layer of palladium nuclei on a TiO<sub>2</sub> coated support, described in Examples 15 and 17 on pages 18 and 19 of Belgian Pat. No. 718,019, is treated for 5 minutes at 35 75° F. in Solution A (see Example 1), washed and dried. A second sample containing an identical nickel image is not treated in a Blix solution and served as a control. A comparison between the sensitometric curves of the nickel image in the untreated sample and the formazan dye image in the treated sample demonstrates the effective conversion of nickel to formazan dye in the blix solution according to our invention.

35 B. A copper image is similarly treated with essentially the same result.

40 Example 13 - A Soluble-dye-forming T-salt Blixes Image Silver Without Retention of a Dye Image

45 A black-and-white processed sample of a negative type, developing out fine-grain gelatinous silver bromoiodide coated film is treated in Solution I (see composition below) at 75° F. Solution I is made by dissolving 2 g. of 2,3,5-tri(p-carboxyethylphenyl)-2H-tetrazolium bromide and 20 g. of ammonium thiosulfate to make 100 ml. of solution having a pH of 7.0. The treated sample is subsequently washed and dried. An inspection of the dried sample shows that it is substantially free of silver and free of formazan dye.

50 Example 14 - The Formazan Image Dyes Generated By the Method According to Our Invention Can Be Chelated to Improve the Dyes' Stability and To Shift Their Spectral Absorption Peaks

55 A first sample of a negative type, developing-out fine-grain gelatinous silver bromoiodide emulsion coated film is flash-exposed, black-and-white developed to a silver density of 0.4 fixed, washed and dried. A second sample is similarly processed and subsequently treated for 3 minutes at 75° F. in Solution J (see composition below), washed and dried. Solution J is made by dissolving the following composition:

|                                                                            |          |
|----------------------------------------------------------------------------|----------|
| 2,5-diphenyl-3-(4,5-dimethylthiazol-2-yl)-2H-tetrazolium bromide           | 0.1 g.   |
| Dimethylformamide                                                          | 5.0 ml.  |
| 10% (NH <sub>4</sub> ) <sub>2</sub> S <sub>2</sub> O <sub>8</sub> Solution | 20.0 ml. |

60 in water to make 45 ml. of solution having a pH of 8.0. Two

additional samples are similarly processed and treated in separate preparations of Solution J which contained, instead of the 20 ml. of water, 20 ml. of 10 percent solutions of the metal ions as shown in Table 11. The spectral absorption peaks ( $\lambda_{max}$ ) of the formazan dyes generated in the above samples are recorded in Table 10.

TABLE 10

| ta Sample | Number | Chelating Agent   | $\lambda_{max}$ | $\mu_{max}$  |
|-----------|--------|-------------------|-----------------|--------------|
| 1         |        | —                 | Control         | 0.4 (silver) |
| 2         |        | None              | 625             | 0.76         |
| 3         |        | $Cd(C_6H_5O_2)_2$ | 655             | 9.74         |
| 4         |        | $Zn(C_6H_5O_2)_2$ | 650             | 0.76         |

## EXAMPLE 15

A composition is made like that in Example 2, but in which the ammonium thiosulfate is replaced by an equimolar amount of sodium thiosulfate. Examples 1 and 9 are then repeated, using the modified solution. Results are obtained that are similar to those obtained in Examples 1 and 9.

## EXAMPLE 16

Examples 2 and 9 are repeated, but using in place of Solution B, a solution made by replacing the ammonium thiosulfate with an equimolar amount of ammonium thiocyanate. Similar results to those in Examples 2 and 9 are obtained.

## EXAMPLE 17

Examples 2 and 9 are repeated, but using in place of Solution A, a solution made by replacing the ammonium thiosulfate with an equimolar amount of 3,6-dithia-1,8-octanediol. Results similar to those of Examples 2 and 9 are obtained.

## EXAMPLE 18

An X-ray film like that described in Example 10 is exposed to an X-ray image, developed in a conventional X-ray film developer, fixed, washed and dried. Fifteen identical samples are taken of the processed X-ray film. One sample is used as a control, while the other samples are each treated by contacting with a different Solution K, L, M, N, O, P, Q, R, S, T, U, V and W (described below). The silver image in each of the treated samples is replaced by a formazan dye image corresponding to the particular T-salt used in the treatment solution of our invention. Solutions K through W are made, each containing 10 g. of ammonium thiosulfate per 100 ml. and 1 g. of the T-salt indicated in the table below:

| Solu- | T-salt                                                                       |
|-------|------------------------------------------------------------------------------|
| K     | 2,3-diphenyl-5-(pyrid-2-yl)-2H-tetrazolium bromide                           |
| L     | 2,3-diphenyl-5-(benzoxazol-2-yl)-2H-tetrazolium chloride                     |
| M     | 2,3-di(4-bromophenyl)-5-(benzothiazol-2-yl)-2H-tetrazolium chloride          |
| N     | 5,5'-dimethyl-3,3'-diphenyl-2,2'-di-(p-phenylene)di(2H-tetrazolium chloride) |
| O     | 2,2',3,3'-tetraphenyl-5,5'-diethylene-di(2H-tetrazolium chloride)            |
| P     | 2,3'-diphenyl-2H-tetrazolium chloride                                        |
| Q     | 3-(p-hydroxyphenyl)-5-methyl-2H-tetrazolium chloride                         |
| R     | 2,3-diphenyl-5-dodecyl-2H-tetrazolium chloride                               |
| S     | 2,3-diphenyl-5-hydroxy-2H-tetrazolium chloride                               |
| T     | 5-amino-2,3-diphenyl-2H-tetrazolium chloride                                 |
| U     | 5-carboxy-2,3-diphenyl-2H-tetrazolium chloride                               |
| V     | 5-benzamido-2,3-diphenyl-2H-tetrazolium chloride                             |
| W     | 5-ethoxycarbonyl-2,3-diphenyl-2H-tetrazolium chloride                        |

## Example 19

A multilayer, multicolor photographic film having a red-sensitized negative-speed gelatino-silver bromoiodide emulsion layer containing a nondiffusible phenolic cyan-dye-forming coupler that was incorporated with a low-boiling solvent (e.g., ethyl acetate), a green-sensitized negative-speed

gelatino-silver bromoiodide emulsion layer containing a nondiffusible 5-pyrazolone magenta-dye-forming coupler that was incorporated with ethyl acetate as solvent, and a blue-sensitive negative-speed gelatino-silver bromoiodide emulsion containing a nondiffusible acetoacetanilido yellow-dye-forming coupler that was incorporated with ethyl acetate as the coupler solvent is sensitometrically exposed and color processed as described in Example 2, Column 12 of U.S. Pat. No. 2,944,900 up to the bleach and fix steps, which are replaced by contacting the developed and washed film with Blix solution described in our Example 13. The blixed film is then washed and dried, leaving the color reproduction made of dyes formed from the incorporated couplers in the color development step and essentially no residual silver.

15 This patent application is being filed simultaneously with another patent application in our names which describes and claims a related invention of ours that is concerned with replacing a metal image with a formazan dye image by contacting the metal image with a solution of a T-salt that contains at least one complexing moiety (on T-salt) that complexes metal so that no external source of complexing agent is required as is required in our invention described and claimed in the immediate patent application.

20 The invention has been described in detail with particular reference to preferred embodiments thereof, but, it will be understood that variations and modifications can be effected within the spirit and scope of the invention.

We claim:

- 30 1. A photographic composition for converting a zero valent metal image into a formazan dye comprising (a) a soluble and diffusible tetrazolium salt and (b) a ligand which produces a silver complex having a smaller cumulative equilibrium constant of  $\beta_2$  than the complex of silver with cyanide ion, such that the combination of said tetrazolium salt and said ligand with a zero valent metal image in the presence of water produces a solution reaction potential of at least +0.01 volt.
- 35 2. A photographic composition for converting a zero valent metal image into a formazan dye comprising (a) a water-soluble, diffusible tetrazolium salt represented by the formulas:



45 whereon  $\text{R}_1$  and  $\text{R}_3$  each represent a group selected from the class consisting of an aryl group and a heterocyclic group;  $\text{R}_2$  represents a member selected from the class consisting of hydrogen, an alkyl group, an aryl group, a heterocyclic group, hydroxyl, carboxyl group, salt of carboxyl group, a carboxy-ester group, an amino group, a carbamyl group, sulfo, a sulfonamido group, a sulfamyl group, the mercapto group and the nitro group;  $\text{X}^{\ominus}$  represents an anion;  $\text{D}$  represents a divalent aromatic group and  $\text{E}$  represents a divalent group selected from the class consisting of an alkylene group, an arylene group and an aralkylene group;  $n$  represents an integer of from 1 to 5; and (b) a metal complexing agent which produces a silver complex having a cumulative equilibrium constant  $\beta_2$  that is at least  $10^3$  times less than said constant for the complex of silver with cyanide ion, such that the combination of said tetrazolium salt and said complexing agent with a zero valent metal image in the presence of

water produces a solution reaction potential of at least +0.01 volt.

3. A composition of claim 2 in which the metal complexing agent is selected from the class consisting of a water-soluble thiosulfate, thiourea, ethylenethiourea, a water-soluble thiocyanate, a water-soluble sulfur containing dibasic acid and a water-soluble diol containing sulfur atoms.

4. A composition of claim 2 in which the tetrazolium salt is 2,3,5-triphenyl-2H-tetrazolium chloride.

5. A composition of claim 2 in which the tetrazolium salt is 2,3,5-tri(p-carboxyphenyl)-2H-tetrazolium bromide.

6. A composition of claim 2 in which the metal complexing agent is a water-soluble thiosulfate.

7. A photographic composition comprising 2,3,5-triphenyl-2H-tetrazolium chloride and ammonium thiosulfate, which combination with a zero valent metal image in the presence of water produces a solution reaction potential of at least +0.01 volt and which metal complexes are water soluble and diffusible.

8. A photographic composition comprising 2,3,5-tri(p-carboxyethylphenyl)-2H-tetrazolium bromide and ammonium thiosulfate which combination with a zero valent metal image in the presence of water produces a solution reaction potential of at least +0.01 volt and which metal complexes are water soluble and diffusible.

9. A photographic composition comprising 2-(benzothiazol-2-yl)-3-phenyl-5-(o-chlorophenyl)-2H-tetrazolium chloride and ammonium thiosulfate, which combination with a zero valent metal image in the presence of water produces a solution reaction potential of at least +0.01 volt and which metal complexes are water soluble and diffusible.

10. A photographic composition comprising 2-(4,5-dimethylthiazol-2-yl)-3,5-diphenyl-2H-tetrazolium bromide and ammonium thiosulfate, which combination with a zero valent metal image in the presence of water produces a solution reaction potential of at least +0.01 volt and which metal complexes are water soluble and diffusible.

11. A process for converting at least a portion of a zero valent metal image to a formazan dye image which comprises contacting said metal image with a water-soluble, diffusible ligand that forms a silver complex with a smaller cumulative equilibrium constant  $\beta_2$  than the complex of silver with cyanide ion, such that the combination of said metal, said tetrazolium salt, said ligand and water produces a solution reaction potential of at least +0.01 volt.

12. A process of converting at least a portion of a zero valent metal image to a nondiffusible formazan dye image which comprises the step of contacting said metal image with an aqueous solution containing (1) a water-soluble, diffusible tetrazolium salt represented by the formulas:



wherein R<sub>1</sub> and R<sub>3</sub> each represent a group selected from the class consisting of an aryl group and a heterocyclic group, R<sub>2</sub> represents a member selected from the class consisting of hydrogen, an alkyl group, an aryl group, a heterocyclic group, hydroxyl, carboxyl group, salt of carboxyl group, a carboxy-ester group, an amino group, an amido group, a carbamyl group, sulfo, a salt of the sulfo group, a sulfonamido group, a sulfamyl group, the mercapto group and the nitro group; X<sup>⊖</sup> represents an anion; D represents a divalent aromatic group and E represents a divalent group selected from the class consisting of an alkylene group, an arylene group and an aralkylene group; n represents an integer of from 1 to 5; and (2) a metal complexing agent which produces a silver complex that has a cumulative equilibrium constant  $\beta_2$  that is at least 10<sup>3</sup> times smaller than said constant for the complex of silver with cyanide ion, such that the combination of said aqueous solution with said metal image produces a solution reaction potential of at least +0.01 volt.

13. A single-step photographic process for converting at least a portion of a zero valent metal image in a hydrophilic colloid layer to a nondiffusible formazan dye image, said process comprising the step of contacting said metal image with an aqueous solution containing (1) a water-soluble, diffusible tetrazolium salt and (2) a metal complexing agent which produces a silver complex having a cumulative equilibrium constant  $\beta_2$  that is at least 10<sup>3</sup> times smaller than said constant for the complex of silver with cyanide ion, such that the combination of said aqueous solution with said zero valent metal produces a solution reaction potential of at least +0.01 volt.

14. A process of claim 11 in which the formazan dye image formed is nondiffusible.

15. A process of claim 11 in which the formazan dye is diffusible.

16. A process for converting a silver image in a gelatin layer to a formazan dye image and removing silver and silver salts comprising the step of contacting said silver image with an aqueous solution containing 10 g. of 2,3,5-triphenyl-2H-tetrazolium chloride and 200 g. of ammonium thiosulfate per liter of solution.

17. A process for converting a silver image in a gelatin layer to a formazan dye image and removing silver and silver salts comprising the step of contacting said silver image with an aqueous solution containing 10 g. of 2,3,5-triphenyl-2H-tetrazolium chloride, 100 g. of ammonium thiosulfate, 10 g. of disodium phosphate, 0 to 0.8 ml. of benzyl alcohol, 0 to 0.1 of ethylene thiourea, 0 to 10 g. of thiourea per liter of solution.

18. A process for converting a silver image in a gelatin layer to a formazan dye image and removing silver and silver salts comprising the step of contacting said silver image with an aqueous solution containing 3-phenyl-5-(o-chlorophenyl)-2H-tetrazolium chloride and 100 g. of ammonium thiosulfate per liter of solution.

19. A process for converting a silver image in a gelatin layer to a formazan dye image and removing silver and silver salts comprising the step of contacting said silver image with an aqueous solution containing 10 g. of 2-(4,5-dimethylthiazol-2-yl)-3,5-diphenyl-2H-tetrazolium bromide and 100 g. of ammonium thiosulfate per liter of solution.

20. A process for converting a silver image in a gelatin layer to a formazan dye image and removing silver and silver salts comprising the step of contacting said silver image with an aqueous solution containing 1 g. of 2,3,5-triphenyl-2H-tetrazolium chloride, 0.2 g. of 2-(4,5-dimethylthiazol-2-yl)-3,5-diphenyl-2H-tetrazolium bromide and 12 g. of ammonium thiosulfate per 120 ml. of solution.

\* \* \* \* \*

UNITED STATES PATENT OFFICE  
CERTIFICATE OF CORRECTIONPatent No. 3,642,478 Dated February 15, 1972Inventor(s) Albert T. Brault and Vernon L. Bissonette

It is certified that error appears in the above-identified patent and that said Letters Patent are hereby corrected as shown below:

Column 2, line 35, that part of formula reading:

.059 should read .059 ;  
d

lines 41-42, "d represents the number of electrons transferred in said reaction;" should be deleted; line 55, after "formulas", ";" should read --:--.

Column 3, line 1, "Carboxyethylphenyl" should read --carboxyethylphenyl--; line 13, "hereto" should read --hetero--; line 40, "carboxyl," (second occurrence) should be deleted.

Column 4, line 8, that part of formula reading "diphenyl" should read --diphenyl--; line 9, that part of formula reading "5hydroxy" should read --5-hydroxy--; line 15, that part of formula reading "2,3diphenyl" should read --2,3-diphenyl--; line 46, that part of formula beginning with "3,5-" is not a part of the preceding formula and should have been placed at the beginning of line 47.

Column 5, line 8, that part of formula reading "-2-quinol-2-yl" should read --2-(quinol-2-yl)--; line 24, that part of formula reading "5sulfo" should read --5-sulfo--; line 53, "acetato" should read --acetate--.

Column 7, line 3, that part of formula reading "CH<sub>2</sub>O(2" should read --CH<sub>2</sub>O)2--; line 3, that part of formula reading "CH<sub>2</sub>OH" should read --CH<sub>2</sub>CH<sub>2</sub>OH--; line 16, that part of formula reading "CH<sub>bo</sub> OH" should read --CH<sub>2</sub>OH--; line 67, "Ma<sub>2</sub>HPO<sub>4</sub>" should read --Na<sub>2</sub>HPO<sub>4</sub>--.

UNITED STATES PATENT OFFICE  
CERTIFICATE OF CORRECTION

Patent No. 3,642,478

Dated February 15, 1972

Inventor(s) Albert T. Brault and Vernon L. Bissonette

- 2 -

It is certified that error appears in the above-identified patent and that said Letters Patent are hereby corrected as shown below:

Column 8, line 20, after "1" and before "of" should be inserted --g---.

Column 9, line 4, that part of formula reading "4,5dimethylthiazd" should read --4,5-dimethylthiazol--; line 23, "1" should read --2--; line 51, after "observation", --is-- should be inserted; line 57, "tg" should be deleted.

Column 10, line 17, "30" should read --77--; line 17, under heading "30 sec." should be inserted --30--; line 30, that part of formula reading "tri henyl" should read --triphenyl--; line 52, "v" should be deleted.

Column 11, line 23, ":" should read --;--; line 28, "17the" should read --17th--

Column 12, line 70, "the 0.1 g." should be deleted and --0.1 g.-- should be placed at the right margin of the column above "5.0 ml."

Column 13, line 11, "ta" should be deleted.

Column 14, line 11, before "described", --I-- should be inserted.

In the Claims:

Column 14, line 34, "of" (first occurrence) should be deleted; line 64, "slat" should read --salt--.

UNITED STATES PATENT OFFICE  
CERTIFICATE OF CORRECTION

Patent No. 3,642,478 Dated February 15, 1972

Inventor(s) Albert T. Brault and Vernon L. Bissonette - 3 -

It is certified that error appears in the above-identified patent and that said Letters Patent are hereby corrected as shown below:

Column 15, line 42, before "ligand", --tetrazolium salt and a-- should be inserted; line 47, "of" (first occurrence) should read --for--.

Column 16, line 2, after "group" (second occurrence), --;-- should be inserted; line 9, after "group", --;-- should be inserted; line 46, "0.8" should read --8.--.

Signed and sealed this 1st day of May 1973

(SEAL)

Attest:

EDWARD M. FLETCHER, JR.  
Attesting Officer

ROBERT GOTTSCHALK  
Commissioner of Patents